



US007781059B2

(12) **United States Patent**  
**Wu et al.**

(10) **Patent No.:** **US 7,781,059 B2**  
(45) **Date of Patent:** **Aug. 24, 2010**

(54) **FIBER COMPOSITION AND FIBER MADE  
FROM THE SAME**

(75) Inventors: **Ru-Yu Wu**, Taoyuan Hsien (TW);  
**Chih-Wei Chu**, Taoyuan Hsien (TW);  
**Shih-Hsiung Chen**, Taoyuan Hsien  
(TW); **Chao-Yuan Chiang**, Taoyuan  
Hsien (TW)

(73) Assignee: **Far Eastern Textile Ltd.**, Taipei (TW)

(\*) Notice: Subject to any disclaimer, the term of this  
patent is extended or adjusted under 35  
U.S.C. 154(b) by 50 days.

(21) Appl. No.: **11/964,333**

(22) Filed: **Dec. 26, 2007**

(65) **Prior Publication Data**

US 2008/0171202 A1 Jul. 17, 2008

(30) **Foreign Application Priority Data**

Jan. 12, 2007 (TW) ..... 96101253 A

(51) **Int. Cl.**

**D02G 3/00** (2006.01)  
**C08K 5/1539** (2006.01)

(52) **U.S. Cl.** ..... **428/373**

(58) **Field of Classification Search** ..... 428/373;  
524/112; 442/409, 361, 364

See application file for complete search history.

(56) **References Cited**

U.S. PATENT DOCUMENTS

4,789,592 A \* 12/1988 Taniguchi et al. ..... 428/373

5,206,080 A \* 4/1993 Tashiro et al. ..... 442/200  
5,607,766 A \* 3/1997 Berger ..... 428/373  
5,994,244 A \* 11/1999 Fujiwara et al. ..... 442/365  
6,174,603 B1 \* 1/2001 Berger ..... 428/373  
6,780,367 B2 \* 8/2004 Pyzik et al. ..... 264/333  
7,025,825 B2 \* 4/2006 Pyzik et al. ..... 106/802  
7,518,064 B2 \* 4/2009 Morioka et al. ..... 174/120 R  
2002/0018895 A1 \* 2/2002 Pyzik et al. ..... 428/373  
2004/0258911 A1 \* 12/2004 Pyzik et al. ..... 428/364  
2005/0148268 A1 \* 7/2005 Tai ..... 442/414  
2007/0160799 A1 \* 7/2007 Nguyen ..... 428/74  
2008/0057309 A1 \* 3/2008 Liu et al. ..... 428/375  
2008/0105454 A1 \* 5/2008 Morioka et al. ..... 174/120 SR  
2008/0260974 A1 \* 10/2008 Morton-Finger ..... 428/17  
2009/0061709 A1 \* 3/2009 Nakai et al. ..... 442/170

FOREIGN PATENT DOCUMENTS

JP 03133625 A \* 6/1991  
JP 03287875 A \* 12/1991  
JP 2849929 B2 \* 1/1999  
JP 2851678 B2 \* 1/1999

\* cited by examiner

Primary Examiner—Cheryl Juska

(74) Attorney, Agent, or Firm—Stephen A Bent; Foley & Lardner LLP

(57) **ABSTRACT**

A fiber modifier for improving thermo-bonding affinity of a composite fiber to a natural fiber includes a blend of maleic anhydride and a copolymer component selected from a copolymer of ethylene and acrylic acid, a copolymer of ethylene and methacrylic acid, and combinations thereof. A core and sheath composite fiber including a sheath component made from a fiber composition that contains the above fiber modifier is also disclosed.

**4 Claims, No Drawings**

## FIBER COMPOSITION AND FIBER MADE FROM THE SAME

### CROSS-REFERENCE TO RELATED APPLICATION

This application claims priority of Taiwanese application no. 096101253, filed on Jan. 12, 2007.

### BACKGROUND OF THE INVENTION

#### 1. Field of the Invention

This invention relates to a fiber composition, more particularly to a fiber composition including a fiber modifier containing a blend of maleic anhydride and a copolymer component.

#### 2. Description of the Related Art

Disposable hygienic absorbent products, such as disposable diapers, generally include a liquid-permeable surface layer, a liquid-impermeable backsheet, and an absorbent layer interposed between the liquid-permeable surface layer and the liquid-impermeable backsheet. The absorbent layer is typically made from an absorbent material that includes natural fibers such as cellulose fluff pulp fibers, cotton fibers, and rayon fibers, and a super absorbent polymer (SAP). After water is absorbed into the absorbent layer, the absorbent material of the absorbent layer tends to expand and become heavy, and results in an uncomfortable feeling. Thus, in addition to the absorbent material, synthetic fibers are incorporated into the absorbent layer so as to form a supportive structure to fix the absorbent material in place.

The synthetic fibers traditionally used for formation of the supportive structure are thermo-bondable bi-component fibers made from polyolefins, polyesters or combinations thereof. Since these traditional thermo-bondable bi-component fibers have a poor thermo-bonding affinity for the natural fibers, the supportive structure formed by these traditional thermo-bondable bi-component fibers is unable to effectively fix the absorbent material in place. In order to improve adhesion between the thermo-bondable bi-component fibers and the natural fibers, a bi-component fiber disclosed in U.S. Pat. No. 5,981,410 (hereinafter referred to as the '410 patent) has been widely used in the market place. Particularly, in the Examples of the '410 parent, the core component of the bi-component fiber is made from polypropylene, and the sheath component of the bi-component fiber includes non-grafted polyethylene and polyethylene grafted with maleic anhydride. The maleic anhydride is used as a modifier for improving the thermo-bonding affinity of the bi-component fiber to natural fibers.

### SUMMARY OF THE INVENTION

The object of the present invention is to provide a new and useful fiber modifier for improving thermo-bonding affinity of a composite fiber to a natural fiber.

According to one aspect of this invention, a fiber modifier includes a blend of maleic anhydride and a copolymer component. The copolymer component is selected from the group consisting of a copolymer of ethylene and acrylic acid, a copolymer of ethylene and methacrylic acid, and combinations thereof.

According to another aspect of this invention, a fiber composition includes polyethylene and a fiber modifier. The fiber modifier contains a blend of maleic anhydride and a copolymer component selected from the group consisting of a

copolymer of ethylene and acrylic acid, a copolymer of ethylene and methacrylic acid, and combinations thereof.

According to yet another aspect of this invention, a core and sheath composite fiber includes a core component and a sheath component. The sheath component is made from a fiber composition including polyethylene and a fiber modifier. The fiber modifier contains a blend of maleic anhydride and a copolymer component selected from the group consisting of a copolymer of ethylene and acrylic acid, a copolymer of ethylene and methacrylic acid, and combinations thereof.

### DETAILED DESCRIPTION OF THE PREFERRED EMBODIMENTS

15 This invention relates to a fiber modifier for improving thermo-bonding affinity of a composite fiber to a natural fiber. The fiber modifier includes a blend of maleic anhydride and a copolymer component selected from the group consisting of a copolymer of ethylene and acrylic acid, a copolymer of ethylene and methacrylic acid, and combinations thereof.

20 In one preferred embodiment, the content of maleic anhydride in the blend ranges from 3% to 4% by weight.

25 In another preferred embodiment, the copolymer component is the copolymer of ethylene and acrylic acid. Preferably, the weight ratio of ethylene to acrylic acid in the copolymer component ranges from 91:9 to 82:18. More preferably, the weight ratio of ethylene to acrylic acid in the copolymer component ranges from 90:10 to 85:15.

30 The copolymer of ethylene and acrylic acid includes, but is not limited to, Nucrel 2806 (the DuPont Company), PRIMACOR 3460 (the Dow Chemical Company), ESCOR5200 (the ExxonMobil Chemical Company), and the like.

35 In yet another preferred embodiment, the copolymer component is the copolymer of ethylene and methacrylic acid. Preferably, the weight ratio of ethylene to methacrylic acid in the copolymer component ranges from 96:4 to 85:15. More preferably, the weight ratio of ethylene to methacrylic acid in the copolymer component ranges from 91:9 to 35:15.

40 The copolymer of ethylene and methacrylic acid includes, but is not limited to, Nucrel 0903 and Nucrel 925 (the DuPont Company), and the like.

45 In addition, non-limiting examples of the natural fiber that may be used for bonding to the composite fiber includes cellulose fibers, such as cotton fibers, Rayon fibers, and cellulose fluff pulp fibers, viscose fibers, and Lyocell, etc.

The preferred embodiment of a fiber composition according to this invention includes polyethylene and a fiber modifier as described in the preceding paragraphs.

50 In one preferred embodiment, the weight ratio of polyethylene to the fiber modifier ranges from 95:5 to 88:12. More preferably, the weight ratio of polyethylene to the fiber modifier ranges from 94:6 to 89:11. If the content of the fiber modifier in the fiber composition is higher than 12% by weight, the spinnability of the resulting core and sheath composite fiber is poor. On the other hand, if the content of the fiber modifier in the fiber component is lower than 5% by weight, the thermo-bonding affinity of the resulting core and sheath composite fiber to the natural fiber is not sufficient.

55 The preferred embodiment of a core and sheath composite fiber according to this invention includes a core component and a sheath component made from a fiber composition as described in the preceding paragraph. In particular, the core component has a melting point higher than that of the sheath component.

60 Preferably, the sheath component of the core and sheath composite fiber has a melting point ranging from 88° C. to 130° C.

Preferably, the core component having a melting point higher than that of the sheath component may be made from a polymer selected from the group consisting of polypropylene (m.p. about 150° C. to 170° C.), polyamide (m.p. about 210° C. to 260° C.), polylactic acid (m.p. about 150° C. to 170° C.), polyester (m.p. about 200° C. to 255° C.), and combinations thereof.

The core and sheath composite fiber may be produced by melt-spinning techniques, and can be incorporated with the natural fibers to form a non-woven fabric web.

The thermo-bonding affinity of the core and sheath composite fiber according to this invention to the natural fibers will increase with an increase in the content of acryl groups in the fiber modifier. The inventors of the present invention found that the improvement in thermo-bonding affinity of the core and sheath composite fiber to the natural fibers is attributed to hydrogen bonding between carboxylic groups derived from maleic anhydride and carboxylic groups of acrylic acid or methacrylic acid of the fiber modifier, and hydrogen bonding between carboxylic groups derived from maleic anhydride and hydroxyl groups of the natural fibers.

In addition, the copolymer component used in the fiber modifier of this invention, i.e., the copolymer of ethylene and acrylic acid, the copolymer of ethylene and methacrylic acid, or combinations thereof, has a melting point ranging from 83 to 101° C., which is lower than the melting point of polyethylene (about 130° C.). Therefore, compared to the conventional modifier, such as grafted polyethylene, the fiber modifier according to this invention can be prepared through blending at a relatively low temperature. In addition, grafting reaction which is required in preparation of the conventional modifier and which is relatively unstable and has to be conducted at a relatively high temperature can be omitted. Hence, the manufacture of the fiber modifier of this invention is relatively economical and controllable.

Preparation examples and test examples are given below to illustrate the present invention in further detail, but the scope of the invention should not be limited to these examples.

#### Preparation of the Fiber Modifier of this Invention

##### Example A1

A copolymer of ethylene and methacrylic acid (Nucrel 925, melt index: 25 g/10 min, methacrylic acid content 15 wt %, m.p. 92° C., DuPont Company), and a reactant mixture of maleic anhydride (UPC Technology Corp.), methyl ethyl ketone (TT-308, obtained from Lison Chemical company Ltd.), and dicumyl peroxide (0529F, obtained from Lison Chemical Company Ltd.) in a ratio of 4:4:0.2 were fed into an inlet section of a twin-screw extruder (Japan Steel Works Company) at feeding rates of 16 kg/hr and 1.3 kg/hr, respectively. The vacuum level of the twin-screw extruder was set to 0.6 kg/cm<sup>2</sup>. The rotating speed of the two screws of the twin-screw extruder was set to 250 rpm.

The composition of the copolymer and the reactant mixture was subsequently moved to a heating section of the twin-screw extruder. The heating section was divided into 1<sup>st</sup> to 13<sup>th</sup> heating zones from the inlet section to an outlet section. The heating temperatures of the 1<sup>st</sup> to 13<sup>th</sup> heating zones were separately set to 92° C., 146° C., 182° C., 185° C., 185° C., 186° C., 191° C., 195° C., 201° C., 204° C., 205° C., 213° C., and 215° C. Thereafter, the melted composition left the twin-screw extruder under a temperature of 220° C. A blend of maleic anhydride and a copolymer of ethylene and meth-

acrylic acid, i.e., the fiber modifier of the present invention, was obtained. Melt index: 12 g/10 min. Melting point: 91.04° C.

##### Example A2

The fiber modifier of Example A2 was prepared in a manner similar to that of Example A1, except that the copolymer of ethylene and methacrylic acid used in Example A1 was replaced with another copolymer of ethylene and methacrylic acid (Nucrel 0903, methacrylic acid content 9 wt %, m.p. 101° C., DuPont company). Melting point of the fiber modifier obtained from this Example was 98.65° C.

##### Example A3

The fiber modifier of Example A3 was prepared in a manner similar to that of Example A1, except that the copolymer of ethylene and methacrylic acid used in Example A1 was replaced with a copolymer of ethylene and acrylic acid (Nucrel 2806, acrylic acid content 18 wt %, m.p. 83° C., DuPont company). Melting point of the fiber modifier obtained from this Example was 82.56° C.

##### Example A4

The fiber modifier of Example A4 was prepared in a manner similar to that of Example A1, except that the copolymer of ethylene and methacrylic acid used in Example A1 was replaced with another copolymer of ethylene and acrylic acid (ESCOR5200, acrylic acid content 15 wt %, m.p. 88° C., ExxonMobil Chemical Company). Melting point of the fiber modifier obtained from this Example was 89.60° C.

##### Contact Angle Test

Four starting materials, i.e., the fiber modifier obtained from Example A1, polyethylene (LH-520, m.p.: 130° C., USI Corporation) grafted polyethylene (AMPLIFY GR204, the Dow Chemical Company) and a copolymer of ethylene and methacrylic acid (Nucrel 925, Dupont Company) without maleic anhydride, were separately pressed with a load of 70 kg/cm<sup>2</sup> by a hydraulic press in a hot mold at 200° C. for 15 minutes, and then cooled in a cold mold for 25 minutes. Four samples SE1 to SE4, which respectively correspond to the four starting materials in the above mentioned order, were obtained. Each of the samples SE1 to SE4 had an area of 10 cm<sup>2</sup> and a thickness of 3 cm. Each of the samples SE1 to SE4 was subjected to a contact angle test using Face contact angle-meter (Model: CA-D, KYOWA Interface Science Co., Ltd.) for five times, and the contact angle value of deionized water to each sample at each time of the test was determined. Average of the contact angle values of the five times of the test for each sample is shown in Table 1. The larger the contact angle value of deionized water to the sample, the higher will be the hydrophobicity of the sample. Furthermore, the higher the hydrophobicity of the sample, the poorer will be the thermo-bonding affinity of the sample to natural fibers that are rich in hydroxyl groups.

TABLE 1

| Sample No.                 | Average of contact angle values |
|----------------------------|---------------------------------|
| SE1 (Example A1)           | 50.7                            |
| SE2 (Polyethylene)         | 88.8                            |
| SE3 (Grafted polyethylene) | 71.3                            |

TABLE 1-continued

| Sample No.                                                                | Average of contact angle values |
|---------------------------------------------------------------------------|---------------------------------|
| SE4 (Copolymer of ethylene and methacrylic acid without maleic anhydride) | 76.7                            |

According to the results shown in Table 1, the contact angle value of deionized water to SE1 is much smaller than those of deionized water to SE2 to SE4. This demonstrates that compared to conventional modifiers, i.e., grafted polyethylene, and copolymer of ethylene and methacrylic acid without maleic anhydride, the fiber modifier obtained from Example A1, i.e., the fiber modifier according to this invention, has a more excellent thermo-bonding affinity to the natural fibers. Thus, when the fiber modifier of this invention is applied to the manufacture of a sheath component of a core and sheath composite fiber, the core and sheath composite fiber thus made can be expected to have improved thermo-bonding affinity.

#### Preparation of a Fiber Composition for a Sheath Component of a Core and Sheath Composite Fiber

#### Examples B1 to B4

Sheath components of the fiber composition of Examples B1 to B4 for use in a core and sheath composite fiber were prepared by mixing the fiber modifier obtained from Example A1 with polyethylene in different ratios as shown in Table 2 below. The fiber modifier obtained from Example A1 and polyethylene were pre-heated prior to the mixing operation at temperatures of 50° C. and 80° C., respectively. Then, the mixtures thus made were separately granulated in an extruder and then melt-spun and drawn into the corresponding sheath components SC1 to SC4 under the conditions (1) and (4) to (11) summarized in Table 5 below.

#### Thermo-Bonding Affinity Test

The sheath components SC1 to SC4 obtained from Examples B1 to B4 were separately placed on a cotton fabric (yarn count: 30 (100% cotton)) fixed on a needle plate, and subsequently subjected to thermosetting treatment together in an oven (model no. R-3, Labortex Co., Ltd.). The thermo-setting treatment was conducted at a melting temperature of 135° C. for 3 minutes. Thereafter, the thermo-bonding affinity of each of the sheath components SC1 to SC4 to the cotton fabric was observed.

The control group was prepared in a manner similar to that of Examples B1 to B4 except that polyethylene was not mixed with the fiber modifier of Example A1. The thermo-bonding affinity of the control group to the cotton fabric was likewise observed. Results of the thermo-bonding affinity test are shown in Table 2 below.

TABLE 2

| Sheath component    | Polyethylene content (wt %) | Fiber modifier content (wt %) | Thermo-bonding affinity |
|---------------------|-----------------------------|-------------------------------|-------------------------|
| SC1                 | 88                          | 12                            | Good                    |
| SC2                 | 89                          | 11                            | Good                    |
| SC3                 | 93                          | 7                             | Good                    |
| SC4                 | 94                          | 6                             | Good                    |
| Control group       | 100                         | —                             | Poor                    |
| Melting temperature |                             | 135° C.                       |                         |

According to the results shown in Table 2, addition of the fiber modifier of this invention will improve the thermo-bonding affinity of the sheath component to the cotton fabric (i.e., the natural fibers).

#### Examples B5 to B7

Sheath components SC5 to SC7 of Examples B5 to B7 were prepared in a manner similar to that of Example B2 (i.e., the weight ratio for polyethylene to the fiber modifier was 89:11), except that the fiber modifiers used in Examples B5 to B7 were separately obtained from Examples A2 to A4.

#### Comparison Between Sheath Component SC2 and SC5 to SC7, and Control Group in Thermo-Bonding Affinity to Natural Fibers

Sheath components SC5 to SC7 were subjected to the thermo-bonding affinity test in a manner similar to that of the sheath component SC2. Results of the thermo-bonding affinity test obtained from the sheath components SC2, SC5 to SC7, and the control group, and acrylic acid or methacrylic acid content of the fiber modifier used therein are summarized in Table 3 for convenience of comparison.

TABLE 3

| Sheath component    | Acrylic acid or methacrylic acid content of the fiber modifier | Thermo-bonding affinity |
|---------------------|----------------------------------------------------------------|-------------------------|
| SC2                 | 15 wt % of methacrylic acid                                    | Very good               |
| SC5                 | 9 wt % of methacrylic acid                                     | Good                    |
| SC6                 | 18 wt % of acrylic acid                                        | Very good               |
| SC7                 | 15 wt % of acrylic acid                                        | Good                    |
| Control group       | —                                                              | Poor                    |
| Melting temperature |                                                                | 135° C.                 |

According to the results shown in Table 3, addition of the fiber modifier of this invention will improve the thermo-bonding affinity of the sheath component to the cotton fabric (i.e., the natural fibers). In addition, the results also demonstrate that the higher the acrylic or methacrylic content of the fiber modifier, the better will be the thermo-bonding affinity of the sheath component to the natural fibers.

#### Thermo-Bonding Affinity Test Under a Lower Melting Temperature

Sheath components SC2, SC5 to SC7 and the control group were subjected to the thermo-bonding affinity test in a manner similar to the abovementioned thermo-bonding affinity test, except that the melting temperature of the oven was lowered to 125° C. Results of the thermo-bonding affinity test obtained from the sheath components SC2, SC5 to SC7, and the control group, and acrylic acid or methacrylic acid content of the fiber modifier used therein are shown in Table 4.

TABLE 4

| Sheath component    | Acrylic acid or methacrylic acid content of the fiber modifier | Thermo-bonding affinity |
|---------------------|----------------------------------------------------------------|-------------------------|
| SC2                 | 15 wt % of methacrylic acid                                    | Very good               |
| SC5                 | 9 wt % of methacrylic acid                                     | Good                    |
| SC6                 | 18 wt % of acrylic acid                                        | Very good               |
| SC7                 | 15 wt % of acrylic acid                                        | Good                    |
| Control group       | —                                                              | Poor                    |
| Melting temperature |                                                                | 125° C.                 |

The results shown in Table 4 demonstrate that, at a lower melting temperature, addition of the fiber modifier according

to this invention is still able to improve the thermo-bonding affinity of the sheath component to the cotton fabric. In other words, by addition of the fiber modifier of this invention, production of the sheath component of the core and sheath composite fiber can be conducted in a power-saving way and at an economical cost.

Preparation of a Core and Sheath Composite Fiber Including a Sheath Component of the Fiber Composition

Example C1

A core and sheath composite fiber was prepared by melt-spinning and drawing techniques. Raw material of the sheath component included the fiber modifier obtained from Example A1 and polyethylene. The fiber modifier of Example A1 and polyethylene were pre-heated to temperatures of 50° C. and 80° C., respectively, and mixed in the same weight ratio as that of Example B2, i.e., 88:11. Raw material of the core component included propylene (6231F, m.p.: 166.1° C., Taiwan Polypropylene Co., Ltd.), which was pre-heated to a temperature of 80° C. The raw material of the sheath component and the raw material of the core component were separately fed into extruders, temperatures of heating zones of which were set according to the conditions (1) and (2) summarized in Table 5 below, so as to form the sheath and core components. The sheath and core components were subsequently fed into a melt-spinning machine (available from Fleissner GmbH, Germany) and a drawing machine (available from Oerlikon Neumag GmbH, Germany) in a weight ratio of 65:35 so as to form the core and sheath composite fiber having a size of 1.5 d×38 mm. The operational conditions of the melt-spinning and drawing machines were set according to the conditions (3) to (7) and (8) to (11) summarized in Table 5 below, respectively.

TABLE 5

| Conditions                                                                                                    |                                                      |
|---------------------------------------------------------------------------------------------------------------|------------------------------------------------------|
| (1) Temperatures set sequentially in five heating zones of the extruder for formation of the sheath component | room temperature, 200° C., 240° C., 240° C., 240° C. |
| (2) Temperatures set sequentially in five heating zones of the extruder for formation of the core component   | 260° C., 260° C., 260° C., 260° C., 260° C.          |
| (3) Weight ratio of the sheath component to the core component                                                | 65%/35%                                              |
| (4) Temperature of heat transfer fluid (Thermolin ®)                                                          | 260° C.                                              |
| (5) Spinneret type                                                                                            | 600 H (for sheath and core components)               |
| (6) Oil peak up percentage (OPU)                                                                              | 0.3                                                  |
| (7) Take-up speed (m/min)                                                                                     | 1350                                                 |
| (8) Draw ratio                                                                                                | 4.2                                                  |
| (9) Drawing temperature                                                                                       | 60° C. to 85° C.                                     |
| (10) Thermosetting temperature                                                                                | 85° C. to 115° C.                                    |
| (11) Drying temperature of filament bundles (Two dryer system)                                                | 113° C.                                              |

Comparative Example 1

A core and sheath composite fiber was made in a manner similar to that of Example C1, except that the sheath component was made only from polyethylene, and that temperatures set sequentially in five heating zones of the extruder for formation of the sheath component were 200° C., 200° C., 240° C., 240° C. and 240° C.

Comparative Example 2

A core and sheath composite fiber was made in a manner similar to that of Example C1, except that the sheath component was made from 89 wt % of polyethylene and 11 wt % of a conventional modifier (Amplify gr204, The Dow Chemical Company), that the conventional modifier was pre-heated to a temperature of 80° C., and that temperatures set sequentially in five heating zones for formation of the sheath component were 200° C., 200° C., 235° C., 240° C. and 240° C.

Comparative Example 3

Commercially available modified polyethylene/polypropylene composite fiber (the CHISSO Corporation) was used as the core and sheath composite fiber of Comparative Example 3.

Example C2

A core and sheath composite fiber was prepared by melt-spinning and drawing techniques. Raw material of the sheath component included 8 wt % of the fiber modifier obtained from Example A1, and 92 wt % of polyethylene. Raw material of the core component included polyester (CSS-910, m.p.: 255° C., Far Eastern Textile Ltd., Taiwan), which was pre-heated to a temperature of 140° C. The raw material of the sheath component and the raw material of the core component were separately fed into extruders, temperatures of heating zones of which were set according to the conditions (1) and (2) summarized in Table 6 below, so as to form the sheath and core components. The sheath and core components were subsequently fed into a melt-spinning machine (available from Fleissner GmbH, Germany) and a drawing machine (available from Oerlikon Neumag GmbH, Germany) in a weight ratio of 55:45 so as to form the core and sheath composite fiber having a size of 2.0 d×38 mm. The operational conditions of the melt-spinning and drawing machines were set according to the conditions (3) to (7) and (8) to (11) summarized in Table 6 below, respectively.

TABLE 6

| Conditions                                                                                                    |                                                             |
|---------------------------------------------------------------------------------------------------------------|-------------------------------------------------------------|
| (1) Temperatures set sequentially in five heating zones of the extruder for formation of the sheath component | room temperature, 200° C., 240° C., 240° C., 240° C.        |
| (2) Temperatures set sequentially in five heating zones of the extruder for formation of the core component   | 295° C., 300° C., 300° C., 305° C., 305° C.                 |
| (3) Weight ratio of the sheath component to the core component                                                | 55%/45%                                                     |
| (4) Temperature of heat transfer fluid (Thermolin ®)                                                          | 260° C. (for sheath component)/280° C. (for core component) |
| (5) Spinneret type                                                                                            | 600 H (for sheath and core components)                      |
| (6) Oil peak up percentage (OPU)                                                                              | 0.3                                                         |
| (7) Take-up speed (m/min)                                                                                     | 1350                                                        |
| (8) Draw ratio                                                                                                | 3.1                                                         |
| (9) Drawing temperature                                                                                       | 50° C. to 90° C.                                            |
| (10) Thermosetting temperature                                                                                | 65° C. to 115° C.                                           |
| (11) Drying temperature of filament bundles (Two dryer system)                                                | 113° C.                                                     |

## Comparative Example 4

A core and sheath composite fiber was made in a manner similar to that of Example C2, except that the sheath component was made only from polyethylene, and that temperatures set sequentially in five heating zones of the extruder for formation of the sheath component were 250° C., 250° C., 255° C., 255° C. and 255° C.

## Comparative Example 5

A core and sheath composite fiber was made in a manner similar to that of Example C2, except that the sheath component was made from 90 wt % of polyethylene and 10 wt % of a conventional modifier (Amplify GR-204, The Dow Chemical Company) and that temperatures set sequentially in five heating zones for formation of the sheath component were 250° C., 250° C., 255° C., 255° C. and 255° C., respectively.

As stated in Example C1 and Comparative Examples 1 and 2, by virtue of addition of the fiber modifier according to this invention, the temperatures set sequentially in five heating zones for formation of the sheath component can start from room temperature. In addition, as stated in Example C1 and Comparative Example 2, the pre-heating temperature required for the fiber modifier of this invention was 50° C., while the pre-heating temperature required for the conventional modifier was 80° C. These facts demonstrate that production of the sheath component of the core and sheath composite fiber can be conducted in a power-saving way and at an economical cost through addition of the fiber modifier of this invention.

Similar results and observations can be obtained from Example C2 and Comparative Examples 4 and 5.

## Evaluation of Physical Properties of Core and Sheath Composite Fiber

Results of the physical properties of the core and sheath composites fibers obtained from Example C1 and Comparative Examples 1 to 3 are shown in Table 7.

TABLE 7

|                                        | Example C1 | Comparative Example 1 | Comparative Example 2 | Comparative Example 3 |
|----------------------------------------|------------|-----------------------|-----------------------|-----------------------|
| Denier (d)                             | 1.61       | 1.60                  | 1.70                  | 1.65                  |
| Length (mm)                            | 38.3       | 38.0                  | 38.0                  | 38.6                  |
| Number of crimp (CN)                   | 13.3       | 12.7                  | 14.3                  | 13.8                  |
| Degree of crimp (CD, %)                | 12.2       | 12.6                  | 14.5                  | 15.0                  |
| Crimp elasticity (CS, %)               | 71.7       | 72.4                  | 80.2                  | 70.3                  |
| Hot air shrinkage (HAS, %) $\leq$ 4.5% | 1.4        | 1.2                   | 2.5                   | 3.1                   |
| Oil peak up percentage (OPU)           | 0.3        | 0.3                   | 0.3                   | —                     |

In addition, results of the physical properties of the core and sheath composites fibers obtained from Example C2 and Comparative Examples 4 and 5 are shown in Table 8.

TABLE 8

|             | Example C2 | Comparative Example 4 | Comparative Example 5 |
|-------------|------------|-----------------------|-----------------------|
| Denier (d)  | 2.76       | 2.4                   | 2.20                  |
| Length (mm) | 40.3       | 39.0                  | 39.0                  |

TABLE 8-continued

|                                        | Example C2 | Comparative Example 4 | Comparative Example 5 |
|----------------------------------------|------------|-----------------------|-----------------------|
| Number of crimp (CN)                   | 13.3       | 12.0                  | 13.0                  |
| Degree of crimp (CD, %)                | 18.3       | 15.5                  | 14.5                  |
| Crimp elasticity (CS, %)               | 82.2       | 80.0                  | —                     |
| Hot air shrinkage (HAS, %) $\leq$ 4.5% | 1.1        | 1.2                   | 1.5                   |
| Oil peak up percentage (OPU)           | 0.3        | 0.3                   | 0.3                   |

According to the results shown in Tables 7 and 8, addition of the fiber modifier of this invention has no adverse effect on the physical properties of the core and sheath composite fiber.

## Thermo-Bonding Test

## Example D1

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 898

## 11

## Example D2

20 g of the core and sheath composite fibers obtained from Example C2 (30 wt %) and Rayon fibers (70 wt %, 2 dx38 mm, Vicunha Textil SA Company) were carded twice in a carding machine. The carded cotton mesh thus made was heated in an oven at 145° C. for 3 minutes so as to form a non-woven fabric web having a basis weight of 100 g/m<sup>2</sup>. The non-woven fabric web was cut into specimens (FD2), each of which has a size of 30 cmx5 cm.

## Comparative Examples 9 to 10

Specimens of the non-woven fabric web of Comparative Examples 9 and 10 (CF9 and CF10) were made in a manner similar to Example D2, except that the core and sheath composite fibers were separately obtained from Comparative Examples 4 and 5.

Breaking strength and elongation of the specimens obtained from Example D2 (FD2) and Comparative Examples 9 and 10 (CF9 and CF10) were determined by a tensile strength test machine (INSTRON-4301) and results are shown in Table 10.

TABLE 10

|      | Breaking strength<br>(kg) | Elongation (%) |
|------|---------------------------|----------------|
| FD2  | 4.0                       | 13.2           |
| CF9  | 0.5                       | 21.6           |
| CF10 | 3.8                       | 15.6           |

According to the results shown in Table 10, specimens of Example D2 (FD2) have a breaking strength almost eight times as high as that of specimens of Comparative Example 9 (CF9). This demonstrates that addition of the fiber modifier of this invention into the sheath component will greatly enhance the thermo-bonding affinity of the core and sheath composite fiber to the natural fiber.

In addition, specimens of Example D2 (FD2) have a breaking strength comparable with or even better than those of the specimens of Comparative Example 10 (CF10). This demon-

## 12

strates that the fiber modifier according to this invention can achieve the same or even better level of thermo-bonding improvement than that of the conventional modifier containing grafted polyethylene.

In view of the foregoing, addition of the fiber modifier of this invention in the fiber composition will enhance the thermo-bonding affinity of the composite fiber thus made to the natural fiber. Besides, addition of the fiber modifier of this invention in the fiber composition will enable the sheath component of the composite fiber to be prepared at a lower temperature. Hence, production cost of the composite fiber can be decreased.

While the present invention has been described in connection with what are considered the most practical and preferred embodiments, it is understood that this invention is not limited to the disclosed embodiments but is intended to cover various arrangements included within the spirit and scope of the broadest interpretation and equivalent arrangements.

What is claimed is:

1. A core and sheath composite fiber, comprising a core component and a sheath component made from a fiber composition, wherein said core component has a melting point higher than that of said sheath component, and wherein said fiber composition comprises polyethylene and a fiber modifier including a blend of maleic anhydride and a copolymer component selected from the group consisting of a copolymer of ethylene and acrylic acid, a copolymer of ethylene and methacrylic acid, and combinations thereof, the weight ratio of polyethylene to said fiber modifier in said sheath component ranging from 95:5 to 88:12.

2. The core and sheath composite fiber of claim 1, wherein the weight ratio of polyethylene to said fiber modifier in said sheath component ranges from 94:6 to 89:11.

3. The core and sheath composite fiber of claim 1, wherein the melting point of said sheath component ranges from 88° C. to 130° C.

4. The core and sheath composite fiber of claim 1, wherein said core component is made from a polymer selected from the group consisting of polypropylene, polyamide, polylactic acid, polyester, and combinations thereof.

\* \* \* \* \*